

# United States Patent [19]

Yoshino et al.

[11] 3,905,876

[45] Sept. 16, 1975

[54] ELECTRORECORDING SHEET

[75] Inventors: **Kimiaki Yoshino**, Neyagawa;  
**Kinichi Adachi**, Takarazuka;  
**Wataru Shimotsuma**, Hirakata;  
**Yoichi Sekine**, Katano; **Toshio Shimizu**, Daito, all of Japan

[73] Assignee: **Matsushita Electric Industrial Co., Ltd.**, Kodoma, Japan

[22] Filed: **Nov. 30, 1973**

[21] Appl. No.: **420,601**

[30] Foreign Application Priority Data

Nov. 30, 1972 Japan..... 47-120898  
Mar. 20, 1973 Japan..... 48-32302

[52] U.S. Cl..... **204/2; 117/36.7; 346/76 R;**  
346/135

[51] Int. Cl..... **B41m 5/20**

[58] Field of Search..... **346/74 CH, 74 E, 76 R,**  
346/135; 204/2, 18 PC; 340/173 CH;  
117/1.7, 36.7, 36.9

[56]

References Cited

UNITED STATES PATENTS

|           |        |                  |         |
|-----------|--------|------------------|---------|
| 3,518,038 | 6/1970 | Spatz .....      | 204/2   |
| 3,642,475 | 2/1972 | Vrancken .....   | 346/135 |
| 3,655,527 | 4/1972 | Curran .....     | 204/2   |
| 3,789,425 | 1/1974 | Matsushima ..... | 346/135 |
| 3,792,481 | 2/1974 | Nagashima.....   | 346/135 |

Primary Examiner—T. M. Tufariello

Attorney, Agent, or Firm—Stevens, Davis, Miller & Mosher

[57]

ABSTRACT

An electrorecording sheet comprises a heat sensitive color forming component which shows color formation or color change upon application of heat energy thereto, cuprous iodide imparting conductivity and a resistance lowering agent for lowering resistance of cuprous iodide by providing a free iodine component to cuprous iodide. When electric current flows across selected areas of the recording sheet, the color forming component in those areas forms color to mark the record.

19 Claims, 8 Drawing Figures



PATENTED SEP 16 1975

3,905,876

SHEET 1 OF 2

FIG. 1



FIG. 2



FIG. 3



FIG. 4



FIG. 5



FIG. 6



FIG. 7



FIG. 8



## ELECTRORECORDING SHEET

The present invention relates to an electrorecording sheet for converting electrical signals directly to visual images adapted to be used in an information recording apparatus such as a facsimile, a character printer, an analog recorder or the like.

Prior art recording materials usable for the same purpose as that of the present invention include a sparking record paper, an electrolytic recording paper or the like.

As is well-known in the art, the sparking record paper consists of a black conductive layer of carbon and an overlying layer comprising a white semiconductive metallic compound and binder material, in which recording images are formed by passing current thereacross to destroy portions of the white layer and spatter them away to expose the conductive layer.

The recording sheet of this type is characterized by a dry system, a high recording speed, low cost and elimination of need of developing and fixing processes, but has a disadvantage in that a considerable amount of smoke and odor are generated upon sparking.

The electrolytic recording sheets are classified in two types, one in which metal ions of a recording electrode react with electrolyte impregnated in the recording paper and the other in which the electrolyte is decomposed by current so that the products therefrom form color. These types of recording sheets are advantageous in that they have high sensitivity and are inexpensive but have the disadvantages of electrode consumption and erosion, relatively short effective preservation period of images and those inherent to wet type recording.

It is an object of the present invention to provide an electrorecording sheet which overcomes the shortcomings of the prior art recording sheets, allows use in a lighted place, can provide recordings of high gradient at high speed, has stable image preservation properties without discoloration or fading, is inexpensive and does not require head replacement or toner replacement.

The electrorecording sheet of the present invention comprises a heat sensitive, color forming component which forms color or changes color upon application of heat energy thereto, cuprous iodide which imparts conductivity to the recording sheet and a support sheet bearing the above components. A record is marked by flowing current across a recording stylus electrode in contact with the recording sheet and a counterelectrode to cause color forming or color change of the heat sensitive color forming component in those selected areas adjacent to the recording stylus, through which areas current has been passed.

The electrorecording sheet of the present invention uses transparent or light yellow cuprous iodide as a conductive material and the heat sensitive color forming component forms color or changes color by flowing electric current. Accordingly, neither a colored layer nor a masking layer is required, and substantially no bad odor, recording sludge and smoke are generated, and the recording sheet of the present invention can be used as a copying base paper utilizing transmitted light. Furthermore, since cuprous iodide is hardly influenced by environmental temperature and humidity, no storage container as required as is necessary in wet type recording sheets and recording can always be carried out under a constant condition.

In the electrorecording sheet of this type, it is desirable that the resistivity of the conductive material be less than several  $\Omega \cdot \text{cm}$ , and when this material is applied on or mixed with a support sheet the surface resistivity of a finished recording sheet be less than several  $\text{K}\Omega$ . This is because, by reducing the surface resistivity a high speed recording of about 3.5 m/sec. can be effected with the applied voltage of 200 – 300 V. In order to reduce the surface resistivity of the recording sheet down to less than several  $\text{K}\Omega$ , as stated above, with cuprous iodide having the resistivity of 10  $\Omega \cdot \text{cm}$  which is produced by the reaction of potassium iodide and copper sulfate, such cuprous iodide must be applied or contained in an amount of about 30 g/m<sup>2</sup>. However, with such a substantial amount of conductive material, the finished recording sheet does not exhibit the nature of a plain paper, makes it difficult to be used in transmitting light recording and the cost of the recording sheet increases.

It is an object of the present invention to overcome the above difficulties by lowering the resistance of cuprous iodide itself and provide an electrorecording sheet exhibiting plain paper properties.

Briefly, the present invention is based on the discovery of the fact that a material which imparts a free iodine component to cuprous iodide is effectively used as resistance lowering agent for lowering the resistance of cuprous iodide.

As the resistance lowering agent, those materials may be used, which by themselves can impart an iodine component such as iodine or compound of iodine such as iodoform, tetraiodomethane, and an oxidizing agent which serves to oxidize cuprous iodide to liberate an iodine component thereof such as potassium permanganate.

It has been known that in an ion crystal having a composition which deviates from a stoichiometric one, a p-type semiconductivity is observed when metal ions are short (or anions are excessive). As an example, it has been known that the conductivity of  $\text{Cu}_2\text{O}$  has a close connection with the content of oxygen and the conductivity increases as the content of oxygen becomes excessive. Chemical analysis shows that in cuprous iodide  $\text{CuI}$  the content of iodine I is excessive compared to the stoichiometric ratio derived from molecular formula, that is, one iodine atom to one copper atom. According to the investigation by Negel et al., there exists a close connection between the conductivity of  $\text{CuI}$  and the iodine pressure and the conductivity increases with the iodine pressure. It is considered that this is because iodine is absorbed in cuprous iodide to produce vacant lattice points of  $\text{Cu}^+$  serving as p-type semiconductor, which in turn increases the conductivity. Therefore, the resistance value of cuprous iodide is influenced by the amount of free iodine.

It has become possible to increase the amount of free iodine by adding the resistance lowering agent to commercially available cuprous iodide to thereby reduce the resistance value of cuprous iodide.

After a number of experiments it has been found that a remarkable result is observed when the amount of excess iodine of cuprous iodide is in the range of 0.05 – 0.2 % by weight, which cuprous iodide is used as the conductive material for the electrorecording sheet. When more iodine is included, the appearance after application of the conductive material is dirty and the excess iodine may fade out during the storage of the re-

corded sheet. Thus, it is inconvenient for practical use. Many materials have been used in experiments for the resistance lowering agent for cuprous iodide and those materials which are listed hereinbelow have been found to be advantageous. Particularly, iodine, iodoform, tetraiodomethane and potassium permanganate showed remarkable effect. For iodoform and tetraiodomethane, it is considered that iodine atoms are liberated and absorbed in cuprous iodide so that the resistance value is reduced. For potassium permanganate, it is considered that it serves as an oxidizing agent for cuprous iodide and removes copper ions from cuprous iodide to produce vacant lattice points of  $Cu^+$  in order to enhance the properties of a p-type semiconductor. In any case, a suitable conductive material for the electrorecording sheet was obtained when the amount of excess iodine of cuprous iodide was in the range of 0.05 - 0.2 % by weight. The cuprous iodide with said resistance lowering agent did not show any change after a test at an environmental temperature of 60°C and under reduced pressure conditions (100 mHg) for 8 hours.

For the other materials listed later, they are advantageous for the resistance lowering agent for cuprous iodide but changes of resistance value were observed after an extended time of storage. No difficulty was encountered, however, in recording at room temperature.

The present invention will now be described in more detail with reference to the accompanying drawings, in which;

FIG. 1 shows a construction of a form of recording sheet in accordance with the present invention;

FIG. 2 illustrates a recording method, and

FIG. 3 - 8 show various forms of construction of recording sheets, in accordance with the present invention.

Referring now to FIGS. 1 and 2 one form of basic construction of the recording sheet of the present invention and recording method are described. In FIG. 1, the recording sheet comprises a support 1 consisting of any one of paper, fabric, glass, plastic material or the like, on which applied is a conductive layer 2 consisting of cuprous iodide having the resistance lowering agent therewith, and an overlying color forming layer 3 including a color forming component which, in response to electric signals, forms color upon application of heat energy thereto. Recording is effected by flowing electric current from an A.C. or D.C. power supply 7, by closing a switch 6, across a recording stylus electrode 4 and a counterelectrode or plane electrode 5 through the color forming layer 3 and the conductive layer 2 so that colored record 8 may be produced on the conductive layer 2 adjacent to the recording stylus electrode 4.

The recording sheet shown in FIG. 1 is a typical example of the construction. Various modifications may be constructed. Examples thereof are shown in FIGS. 3 - 8.

The recording sheet shown in FIG. 3 comprises a single layer 10 consisting of a heat sensitive color forming component and cuprous iodide, formed on a surface of the support 1.

The recording sheet shown in FIG. 4 comprises a conductive layer such as aluminum vapor deposition layer 11 formed on the support 1 similar to that shown in FIG. 1; and a conductive layer 2 of cuprous iodide

and a color forming layer 3 successively formed thereon.

The recording sheet shown in FIG. 5 comprises a conductive layer 12 of carbon on a surface of the support 1 and an overlying layer 10 including a heat sensitive color forming component and cuprous iodide.

The recording sheet shown in FIG. 6 uses a carbon impregnated paper 13 in place of the support 1 shown in FIG. 3.

The recording sheet of FIG. 7 comprises a cuprous iodide impregnated paper 14 as a support and a color forming layer 3 thereon.

The recording sheet of FIG. 8 is formed by a paper in which cuprous iodide and heat sensitive color forming component are impregnated together.

Examples 1 and 2 described later are in accordance with the construction of FIG. 1 and the examples 3 through 7 are in accordance with the constructions of FIGS. 3 through 7, respectively.

Materials suitable for use in the present invention are given below:

1. Heat sensitive color forming material

Those which form color in response to heat energy upon flowing current. They include

- combination of color forming dye such as crystal violet lactone and color forming agent of phenolic acidic material such as bisphenol A,
- organic spot reagent and organic metal, and
- redox indicator. These materials are dispersed in binder material to form color forming component.

a-1. Color-forming dye;

Generally, the color-forming dye used in a leuco body of triphenylmethane type dye represented by the below-mentioned general formula (I) or a leuco body of fluoran type dye represented by the below-mentioned general formula (II).



wherein  $R_x$ ,  $R_y$  and  $R_z$  are individually a hydrogen or halogen atom, or a hydroxyl, alkyl, nitro, amino, dialkylamino, monoalkylamino or aryl group; and  $Z$  is an atom necessary to form a heterocyclic ring, and is O or S.

Concrete examples of the above-mentioned compounds are as shown below. Compounds of the formula (I):

- 3,3-Bis(p-dimethylaminophenyl)-phthalide
- 3,3-Bis(p-dimethylaminophenyl)-6-dimethylaminophthalide (Crystal Violet Lactone)
- 3,3-Bis(p-dimethylaminophenyl)-6-aminophthalide
- 3,3-Bis(p-dimethylaminophenyl)-6-nitrophthalide
- 3,3-Bis(p-dibutylaminophenyl)-phthalide

3,3-Bis(p-dimethylaminophenyl)-4,5,6,7-tetra-chlorophthalide  
Compounds of the formula (II):

- 3-Dimethylamino-6-methoxyfluoran
- 7-Acetamino-3-dimethylaminofluoran
- 3-Dimethylamino-5,7-dimethylfluoran
- 3-Diethylamino-5,7-dimethylfluoran
- 3,6-Bis- $\beta$ -methoxyethoxyfluoran
- 3,6-Bis- $\beta$ -cyanoethoxyfluoran

Other lactam compounds:

- 9-p-Nitroanilino-3,6-bis(diethylamino)-9-xanthenyl-o-benzoic acid lactam (Rhodamin B lactam)
- 9-p-Nitroanilino-3,6-bis(dimethylamino)-9-thio-xanthenyl-o-benzoic acid lactam

The above-mentioned dye bases are effectively used. They are scarcely soluble in water, and can be pulverized to fine particles of less than 10 microns in size.

a-2. Color-forming agent:

Preferable as the color-forming agent capable of forming a dye by chemical reaction with the color-forming dye mentioned in the preceding item (a-1) is a phenolic compound or an organic acid. It is desirable that the said compound or acid is solid at room temperature and can liquefy or vaporize at about 70°C.

i. Examples of the phenolic compound are as follows; 3,5-xylenol, thymol, 4-tert-butylphenol, 4-hydroxyphenoxide, methyl-4-hydroxybenzoate, 4-hydroxyacetophenone,  $\alpha$ -naphthol,  $\beta$ -naphthol, catechol, hydroquinone, resorcinol, 4-tert-octylcatechol, 4,4'-sec-butylidenediphenol, 2,2'-dihydroxydiphenyl, 2,2'-methylenebis(4-methyl-6-tert-butylphenol), 2,2'-bis(4-hydroxyphenyl)-propane, 4,4'-isopropylidenebis-(2-tert-butylphenol), 4,4'-sec-butylidenediphenol, pyrogallol and 4,4'-isopropylidenediphenol.

ii. Examples of the organic acid are as follows:

Stearic, gallic, benzoic, salicylic, succinic, 1-hydroxy-2-naphthoic, 2-hydroxy-p-tolue, o-hydroxybenzoic, m-hydroxybenzoic, p-hydroxybenzoic and 4-hydroxyphthalic acids.

b. Organic spot reagent and organic metal salt:

The organic spot reagent referred to herein is a compound capable of being colored or discolored by reaction with metal ions. At present, a large number of such compounds are known. In the present invention, however, there is utilized the phenomenon that at least one of the organic spot reagent and the metal used in combination therewith is melted due to the heat energy generated at the time of application of electric current and the two react with each other to form a color. It is therefore desirable that one of the two which is lower in melting point is solid at below 70°C. and has a melting point of 150°C. or less. In this respect, metallic soap is most preferable as the organic metal salt. Combinations of the organic spot reagent and the metal are as follows:

1. Organic spot reagent: Metal:

- Diphenylthiocarbazide: Cu, Fe, Mg or Hg
- Dimethylglyoxime: Cu, Fe or Ni
- Benzoquinone: Cu
- 8-Hydroxyquinoline: Cd, Cu, Fe, Pb, Mn, Ni or Zn
- Dinitrophenylcarbazide: Cd
- Rhodanine: Cu or Hg
- Diphenylthiocarbazone: Cu, Ba, Co, Fe, Pb, Hg or Zn
- Diphenylcarbazone: Co, Cu, Pb, Mb, Mn, Hg, Ni or Zn

Dithiooxamine: Co, Cu, Pb or Ni

2-Mercapto-4-phenylthiazole: Co or Pb

3,5-Dimethylpyrazole: Co

$\alpha$ -Naphthylamine-dithiocarbamic acid: Co or Fe

Benzidine: Cu, Pb or Mn

p-Dimethylaminobenzylidene rhodanine: Cu, Fe, Mg or Hg

Salicylaldoxime: Cu or Pb

Triphenyl thiophosphate: Ni

p,p'-Tetramethyl-diaminodiphenylmethane: Pb or Mn

Anthranilic acid: Zn

Diphenylbenzine: Zn

Catechol: Fe

Gallic acid: Fe

Dihydroxynaphthalene: Fe

Alizarine: Cu

Quinalizarin: Cu

ii. Organic metal salt:

As the organic metal salt, a metallic soap having the aforesaid metal ions is effective. Typical examples of the combinations of organic spot reagents with organic metal salts, and color tones of colors developed by use of said combinations, are shown below.

Organic spot reagent: Organic metal salt (Color tone of developed color)

Dimethylglyoxime: Nickel stearate (Pink)

Benzoinoxime: Copper myristate (Yellowish green)

Dithiooxamide: Nickel stearate (Purple)

8-Hydroxyquinoline: Iron oleate (Black)

Gallic acid: Ferric stearate (Black)

Alizarin: Copper oleate (Purplish red)

Quinalizarin: Copper oleate (Purplish red)

Diphenylcarbazone: Copper stearate (Red)

Diphenylcarbazone: Cadmium stearate (Red)

Diphenylcarbazone: Copper myristate (Purple)

Diphenylcarbazone: Zinc palmitate (Deep red)

Diphenylthiocarbazide: Mercuric stearate (Purple)

Diphenylthiocarbazide: Lead myristate (Deep red)

c. It has been found that a substance, which has heretofore been known as redox indicator, forms a color in the vicinity of recording stylus at the time of application of electric current, and it has been confirmed that said substance is effective as a color-forming material for use in electrorecording paper. The redox indicator referred to herein is a substance which is colored or discolored due to oxidation with the heat generated at the time of application of electric current, and is a leuco body is preferable in view of the whiteness of the background. Examples of the redox indicators used in the present invention, and color tones of colors developed by said indicators, are shown below.

Leucoethyl Nile Blue (Blue)

Leucomethyl Capryl Blue (Blue)

Leucotolidine Blue (Purple)

Leucodiphenylamine (Purple)

Leuco-N-methyldiphenylamine-p-sulfonic acid (Reddish purple)

Leucophenylanthranilic acid (Reddish purple)

Triphenyltetrazolium chloride (Red)

Methylviologen (Purple)

Leucosafanine T. (Red)

Leucoindigosulfonic acid (Blue)

Leucophenosafanine (Red)

Leucomethylene Blue (Blue)

- Leucodiphenylbenzidine (Purple)  
 Leucoerioglucine A (Yellowish green to Red)  
 Leuco-p-nitrodiphenylamine (Purple)  
 Leuco-malachite Green (Green)  
 2. Resistance lowering agent for cuprous iodide  
 a. Iodine  
 b. Iodine compound . . . . . iodoform, tetraiodomethane, iodine salt, periodate, iodate, hypoiodate  
 c. Peroxide . . . . . hydrogen peroxide, sodium peroxide, barium peroxide  
 d. Oxyacid salt . . . . . hypochlorite, chlorate, perchlorate, bromate  
 e. Peroxo acid . . . . . peroxy-disulfate, peroxy-sulfuric acid, peroxyphosphoric acid  
 f. Permanganate . . . . . permanganic acid, potassium permanganate, sodium permanganate, calcium permanganate, etc.

## 3. Binder

In order to disperse in the state of fine particles the color forming dye, color-forming agent, organic spot reagent and organic metal salt used in the color-developing layer, and/or cuprous iodide and resistance lowering agent, and to impart bonding ability thereto, there is used a binder. Since most of the above-mentioned color-forming dyes, color-forming agents, organic spot reagents and cuprous iodide are water-insoluble, the use of a water-soluble binder is effective. Further, the water-soluble substance has such characteristics that it is easily handled and treated at the time of production of recording paper.

## i. Water-soluble binder:

Examples of the water-soluble binder include hydroxyethyl cellulose, carboxymethyl cellulose, methoxy cellulose, polyvinyl alcohol, polyvinyl pyrrolidone, polyacrylamide, polyacrylic acid, gelatin, starch, and gum arabic.

## ii. Water-insoluble binder:

As the binder, an organic solvent-soluble binder may also be used. In case a binary system comprising, for example, a color-forming dye and a color-forming agent, is used as the thermorecording material of the color-developing layer, the two components should individually be dispersed in the form of fine particles into the binder. If either one of the two components is dissolved in a solvent used to dissolve the binder, a color formation reaction to deprive its function as a recording medium takes place at the time of mixing of the two. Accordingly, solvents for the binder mentioned herein are necessarily limited depending on the kind of color-forming components.

Concrete examples of the water-insoluble binder are natural rubber, synthetic rubbers, chlorinated rubbers, alkyd resins, styrene-butadiene copolymers, polybutyl methacrylate, low molecular weight ethylene polymers, low molecular weight styrene polymers, polyvinyl butyral, phenolic resins and nitrocellulose.

## EXAMPLE 1

Mixed with 200 parts by weight of aqueous solution containing 1 % by weight of polyvinyl alcohol (PVA 124 prepared by KURARE Co., Ltd.) was 200 parts by weight of cuprous iodide (prepared by KANTO CHEMICAL Co., Ltd.), and they were milled and mixed by a mixer for two hours. During this process, 1 ml of aqueous solution containing 2 % by weight of po-

tassium permanganate was added. The dispersion solution thus formed is referred to as solution A. The dispersion solution A was applied on an artificial paper by a wire bar conditioned to form a coating layer of 8 microns in thickness (15 g/m<sup>2</sup> in application quantity). The surface resistivity thereof was  $3.5 - 4.5 \times 10^3 \Omega$ . When KMnO<sub>4</sub> was removed from the solution A, the surface resistivity was  $2 - 5 \times 10^5 \Omega$ . Thus, it is clear that the surface resistivity was considerably reduced by the addition of KMnO<sub>4</sub> as the resistance lowering agent to CuI. With a given amount of application, it is possible to use lower recording voltage since the surface resistivity is lower, or with less amount of application it is possible to obtain a desired surface resistivity, saving the cost and giving a more plain paper like property.

Next, mixed with 200 parts by weight of aqueous solution containing 1 % by weight of polyvinyl alcohol was 35 parts by weight of 3,3-bis(p-dimethylaminophenyl)-6-dimethylaminophthalide as color forming dye, and they were milled and mixed for 48 hours in a vessel of 500 ml inner volume. The dispersion solution thus formed is referred to as solution B. In the solution B, the color forming material scarcely dissolved but dispersed in the form of fine particles of no greater than 5 microns. In addition to the solution B, added to 200 parts by weight of aqueous solution containing 10 % by weight of polyvinyl alcohol was 35 parts by weight of 4,4'-isopropylidenediphenol as color forming agent, and they were milled and mixed in a ballmill for 48 hours to prepare a dispersion solution hereinafter referred to as solution C. The color forming agent in the solution C also dispersed in the form of fine particles of no greater than 5 microns. Since the particles are surrounded by polyvinyl alcohol there is no direct contact between the particles. 15 parts by weight of the solution B and 100 parts by weight of the solution C were measured and mixed together while agitating. The resulting solution is referred to as solution D. Then the solution D was applied to the artificial paper on which the solution A had previously been applied, by a wire bar conditioned to provide a coating layer of about 5 microns in thickness. The paper was then dried to form a electrorecording sheet. The surface resistivity of the recording sheet thus formed was 4.2 KΩ and could provide a sharp record having a reflective optical density of 0.88 by using recording voltage of 300 V. Furthermore, it was possible with this recording sheet to carry out transmitted light copying.

The relationship between the amount of KMnO<sub>4</sub> added when the solution A was applied and the surface resistivity under the above conditions is listed below.

| KMnO <sub>4</sub> /CuI                                   | No addition | 1/10 <sup>5</sup> | 1/10 <sup>4</sup> | 1/10 <sup>3</sup> | 1/10 <sup>2</sup> | 1/10 |
|----------------------------------------------------------|-------------|-------------------|-------------------|-------------------|-------------------|------|
| Surface resistivity after application of solution A (KΩ) | 50          | 25                | 4                 | 25                | 100               | 800  |

When the amount of addition exceeded 1/10<sup>2</sup>, the solution became reddish and the conductivity reduced because the amount of cuprous oxide increased.

## EXAMPLE 2

Added to 200 parts by weight of hydroxyethylcellulose (Cellosise WP-300H prepared by Union Carbide International Co.) was 200 parts by weight of cuprous iodide and 0.5 parts by weight of iodine (prepared by KANTO CHEMICAL Co., Ltd.), and they were milled and mixed by a mixer for 2 hours. The dispersion solution thus prepared is referred to solution E. The dispersion solution E was then applied on an artificial paper by a wire bar conditioned to provide a coating layer of 10 microns in thickness, and the paper was dried. The surface resistivity after application was  $2 - 3 \times 10^3 \Omega$ . When the iodine was not added as the resistance lowering agent, the surface resistivity was  $2 - 5 \times 10^5 \Omega$ . Thus, it is clear that the surface resistivity was considerably reduced by the addition of iodine. Recording under a lower recording voltage can thus be attained.

Next, added to 100 parts by weight of aqueous solution containing 5 % by weight of hydroxyethylcellulose (Cellosise WP-09L) was 20 parts by weight of 3,3 bis(-p-dimethylaminophenyl)-6-dimethylaminophthalide as color forming material, and they were milled and mixed in a ballmill for 48 hours. The solution thus prepared is referred to as solution F. In addition, added to 100 parts by weight of aqueous solution containing 5 % by weight of hydroxyethylcellulose (Cellosise WP-09L) was 35 parts by weight of 4,4'-isopropylidenediphenol as color forming agent, and they were milled and mixed in a ballmill for 48 hours. The solution thus prepared was referred to as solution G.

15 parts by weight of the solution F and 100 parts by weight of the solution G were mixed and the mixture was applied onto the artificial paper on which the solution E had previously been applied, by a wire bar conditioned to provide a coating layer of about 5 microns in thickness. The paper was then dried to form an electorecording sheet. The surface resistivity of the electorecording sheet thus formed was  $3.8 \text{ K} \Omega$  and could provide recording having reflective optical density of 0.91 using the recording voltage of 300 volts.

## EXAMPLE 3

Added to 100 parts by weight of aqueous solution containing 1 % by weight of polyvinyl alcohol were 100 parts by weight of cuprous iodide and 1 part by weight of iodoform, and they were milled and mixed in a ballmill for 48 hours. The dispersion solution thus prepared is referred to as solution H. Next, added respectively to 100 parts by weight of aqueous solution containing 10 % by weight of polyvinyl alcohol were 30 parts by weight of ferric stearate and 30 parts by weight of gallic acid and separate ballmills for 24 hours. 50 parts by weight of both mixture were mixed to prepare solution I. 100 parts by weight of the solution H and 30 parts by weight of the solution I were mixed by a mixer and applied onto a paper with the thickness of 15 microns. It was then dried to form a light yellow recording sheet. The surface resistivity of the recording sheet was  $1.45 \times 10^4 \Omega$  and a sharp, dark gray record having reflective optical density of 0.80 was obtained at the recording voltage of 300 volts. The structure of the recording sheet is shown in FIG. 3. A color forming conductive layer 10 is provided on the paper 1.

The recording sheets were prepared with varying amounts of iodoform addition to cuprous iodide in the

solution H to determine the value of the recording voltage at which the reflective optical density of the record trane showed 0.80. The result is given below.

| 5  | Solution H                       |                            | Recording voltage |
|----|----------------------------------|----------------------------|-------------------|
|    | Cuprous iodide (parts by weight) | Iodoform (parts by weight) | (V)               |
| 10 | 100                              | 0                          | 820               |
|    | 100                              | 0.1                        | 400               |
|    | 100                              | 0.5                        | 380               |
|    | 100                              | 0.8                        | 340               |
|    | 100                              | 1                          | 300               |
|    | 100                              | 2                          | 280               |
|    | 100                              | 4                          | 250               |
|    | 100                              | 5                          | 250               |

As seen from the above table, the surface resistivity of the recording sheet could be reduced by adding iodoform to cuprous iodide to provide a record having a sufficient density at a relatively low recording voltage.

## EXAMPLE 4

Added to 100 cc of toluene solution containing 10 % by weight of copolymer of styrene and butadiene at the ratio of 85 : 15 were 100 grams of cuprous iodide and 0.5 grams of tetraiodomethane, and they were milled and mixed in a ballmill for 48 hours. The dispersion solution thus prepared was applied onto an aluminum deposited paper by a wire bar conditioned to provide a coating layer of 15 microns, and the paper was dried. The surface resistivity of the applied paper was  $4.3 \times 10^4 \Omega$ .

Next, added to 200 parts by weight of aqueous solution containing 10 % by weight of polyvinyl alcohol was 35 parts by weight of 3-dimethylamino-6-methoxyfulorane as color forming material, and they were milled and mixed in a ballmill for 48 hours, 10 parts by weight of this mixture, 10 parts by weight of the solution C defined in the Example 1 and 5 parts of the dispersion solution of cuprous iodide including tetraiodomethane were mixed together and then applied onto said conductive layer by a wire bar conditioned to provide a coating layer of 10 microns in thickness. The structure of the recording sheet thus formed is shown in FIG. 4. Aluminum deposited layer 11 is formed on the paper 1, and a conductive layer 2 and a color forming layer 3 are formed thereon. The surface resistivity was  $8.3 \times 10^3 \Omega$  and sharp, red record having the reflective optical density of 0.85 was obtained at the recording voltage of 350 V. When tetraiodomethane was not added, the recording sheet prepared otherwise under the same conditions showed the surface resistivity of  $6 \times 10^4 \Omega$  and provided the record having reflective optical density of 0.35 at the recording voltage of 600 V.

## EXAMPLE 5

60 Amorphous carbon 100 parts by weight  
Styrene low polymer 10 parts by weight  
Toluene 100 parts by weight } Solution J

The solution J above was milled and mixed in a ballmill for 24 hours and then applied onto a white paper to form a conductive layer of 10 micron thickness when dried. The surface resistivity of the conductive layer was 250 - 500  $\Omega$ .

Next, 10 parts by weight of leuco Malachite Green, 100 parts by weight of cuprous iodide, 0.2 parts by weight of sodium peroxide, 5 parts by weight of polystyrene sodium sulfonate and 130 parts by weight of water were milled and mixed for 24 hours and then the mixture was applied onto said conductive layer to form a coating layer of 10 micron thickness when dried. A light yellow recording sheet was obtained. When a recording stylus was scanned with a D.C. voltage of 40 volts being applied, a green recording trace was produced. When sodium peroxide was not added as the oxidizing agent, recording was not attained unless a recording voltage higher than 70 volts was applied. FIG. 5 shows the structure of the recording sheet. Carbon layer 12 and color forming conductive layer 10 are formed on the paper 1.

## EXAMPLE 6

|                                      |                      |            |
|--------------------------------------|----------------------|------------|
| Copper palmitate                     | 25 parts by weight   | Solution K |
| Aqueous solution containing 10 % PVA | 100 parts by weight  |            |
| Diphenylcarbazone                    | 25 parts by weight   | Solution L |
| Aqueous solution containing 10 % PVA | 100 parts by weight  |            |
| Cuprous iodide                       | 1000 parts by weight |            |
| Perxo-sulfuric acid                  | 1 part by weight     | Solution M |
| Aqueous solution containing 5 % PVA  | 1000 parts by weight |            |

The above three solutions were respectively milled and mixed for 24 hours, and 15 parts by weight of the solution K, 15 parts by weight of the solution L and 100 parts by weight of the solution M were mixed together and applied onto a conductive paper (having the surface conductivity of  $250 \Omega$ ) including 40 % of carbon fiber to form a coating layer of 10 micron thickness to complete a electrorecording sheet.

When perxo-sulfuric acid was not added, no record was obtained at the recording voltage of 100 V, but when it was added, red record was obtained at the recording voltage of 45 V. The structure of the recording sheet thus formed is shown in FIG. 6. Color forming conductive layer 10 is formed on a carbon impregnated paper 13.

## EXAMPLE 7

Bleached sulfite pulp was beaten thoroughly by a beater. Added to the resulting paper base solution were a sizing agent and 1000 parts by weight of cuprous iodide in the form of fine particles and 1 part by weight of iodine. The paper material was then papered by a cylinder paper machine so that a paper thickness of  $45 \text{ g/m}^2$  was obtained. In this case, since a considerable amount of the conductive material together with the sizing agent flows into white water during the papering process, the white water was flowed back to the paper material preparation process to control the amount of addition so that the conductive material was kept at 6.0 % by weight with respect to the weight of the paper.

Applied onto said paper was the solution D in a manner similar to that explained in the example 1 to form an electrorecording sheet. The structure thereof is shown in FIG. 7.

Color forming layer 3 is formed on a paper 14 including a conductive component.

With this recording sheet, a blue record having the reflective optical density of 0.4 was obtained at the recording voltage of 600 V. When iodine was not added at the resistance lowering agent, no record was obtainable at 600 V.

## EXAMPLE 8

In the process of the Example 7, the paper material was papered so that 6.0 % by weight of cuprous iodide and 2.0 % by weight of leuco Methylene Blue were included. At this time, periodate was added at  $1/10^4$  parts by weight with respect to cuprous iodide as the resistance lowering agent for cuprous iodide. The recording sheet thus prepared could provide a blue record having the reflective optical density of 0.3 at the recording voltage of 600 V. When periodate was not added, no record was obtainable at the recording voltage of 600 V. FIG. 8 shows the structure of the recording sheet, wherein a conductive component and color forming component are impregnated in the paper.

What is claimed is:

1. An electrorecording sheet comprising a heat sensitive color forming component for forming color or changing its color upon application of heat energy thereto, cuprous iodide for imparting conductivity and a support for carrying the above components, said electrorecording sheet for providing a recorded mark when electric current is flowed therethrough in selected areas thereof, by the fact that the heat sensitive color forming component in said selected areas forms color or changes its color, said sheet additionally comprising a resistance lowering agent for providing said cuprous iodide with a free iodine component to lower resistance of said cuprous iodide.

2. An electrorecording sheet according to claim 1, wherein said resistance lowering agent is a material capable of providing its own iodine component.

3. An electrorecording sheet according to claim 1, wherein said resistance lowering agent is an oxidizing agent for oxidizing cuprous iodide to liberate an iodine component.

4. An electrorecording sheet according to claim 2, wherein said material for providing an iodine component is iodine.

5. An electrorecording sheet according to claim 2, wherein said material for providing an iodine component is a compound of iodine.

6. An electrorecording sheet according to claim 3, wherein said oxidizing agent includes at least one material selected from the group consisting of peroxide, oxyacid salt and perxo acid.

7. An electrorecording sheet according to claim 3, wherein said oxidizing agent is permanganate.

8. An electrorecording sheet according to claim 1, wherein said heat sensitive color forming component is a combination of a leuco body of tri-phenylmethane dye or a leuco body of fluorane dye and organic acid or phenolic material.

9. An electrorecording sheet according to claim 1, wherein said heat sensitive color forming component is a combination of metallic salt and an organic spot reagent which rapidly reacts with metal ions of said metallic salt to provide a reaction product having appreciable visual change, one of said two materials which has

the lower melting point has a melting point of 70° – 150°C.

10. An electrorecording sheet according to claim 1, wherein said heat sensitive color forming component is a leuco body of redox indicator.

11. An electrorecording sheet according to claim 1, wherein said cuprous iodide and said resistance lowering agent are dispersed in binder material and applied as a conductive layer on said support, and said heat sensitive color forming component is dispersed in binder material and applied as a color forming layer on said conductive layer.

12. An electrorecording sheet according to claim 1, wherein said cuprous iodide, said resistance lowering agent and said heat sensitive color forming component are dispersed in binder material and applied on said support.

13. An electrorecording sheet according to claim 11, wherein said support is made of one material selected from the group consisting of paper, fabric, plastic film, 20 glass, carbon impregnated paper, metal deposited paper and carbon applied paper.

14. An electrorecording sheet according to claim 12, wherein said support is made of one material selected from the group consisting of paper, fabric, plastic film, 25 glass, carbon impregnated paper, metal deposited paper and carbon applied paper.

15. An electrorecording sheet according to claim 11, wherein said color forming layer includes cuprous iodide.

16. An electrorecording sheet according to claim 15,

wherein said color forming layer further includes a resistance lowering agent.

17. An electrorecording sheet according to claim 1, wherein said support is formed by a fiber impregnated member in which cuprous iodide and a resistance lowering agent are impregnated, said a heat sensitive color forming component is dispersed in binder material and applied as a color forming layer on said support.

18. An electrorecording sheet according to claim 1, 10 wherein said support is formed by fiber impregnated member in which cuprous iodide, resistance lowering agent and heat sensitive color forming component are impregnated.

19. An electrorecording sheet, comprising:  
a heat sensitive color forming component for forming color or changing color upon the application of heat energy thereto;  
cuprous iodide for imparting electrical conductivity to said sheet;  
a resistance lowering agent for providing said cuprous iodide with a free iodine component for lowering the electrical resistance of the cuprous iodide, and  
a support for said component, cuprous iodide and agent; said sheet being capable of providing a recorded mark when an electric current is flowed through selected areas thereof, thereby causing said heat sensitive color forming component to form a color in said selected areas.

\* \* \* \* \*